

Patented Dec. 12, 1922.

1,438,590

# UNITED STATES PATENT OFFICE.

CHARLES N. FORREST, OF RAHWAY, NEW JERSEY, ASSIGNOR TO THE BARBER ASPHALT PAVING COMPANY, OF PHILADELPHIA, PENNSYLVANIA, A CORPORATION OF WEST VIRGINIA.

## FLOTATION PROCESS FOR METALLIC SEPARATION.

No Drawing.

Application filed November 10, 1920. Serial No. 423,162.

To all whom it may concern:

Be it known that I, CHARLES N. FORREST, a citizen of the United States, residing at Rahway, in the county of Union and State 5 of New Jersey, have invented certain new and useful Improvements in Flotation Processes for Metallic Separation, whereof the following is a specification.

My invention comprises a novel flotation 10 process for metallic separation, characterized by the use of a liquid hydrocarbon distillate from the solid native bitumen known as gilsonite. This present application is a continuation in part of my prior application, 15 Serial No. 195,721, of October 10, 1917, entitled "Liquid hydrocarbon," and is filed pursuant to a requirement for division of said prior application made by the United States Patent Office under Rule 42 20 of its Rules of Practice.

The flotation process consists essentially in mixing pulverized metallic ores with water and oil,—or, more commonly, with water and a mixture of different oils,—and 25 then frothing such mixture by agitating or aerating it. The froth collects the metallic particles and rises to the surface of the mixture, while the gangue of non-metallic particles sinks to the bottom. The floating 30 metal-bearing froth flows off from the mixing tank and is treated elsewhere in a suitable manner for the recovery of its metal constituents. The efficiency of any particular oil (or mixture of oils) in flotation is 35 determined, therefore, by the amount of metal it removes from the gangue. As flotation or froth-producing reagents, there have hitherto been used oils produced in the distillation of petroleum; coal or wood tars 40 or products; and mixtures of petroleum or creosote with pine oil or eucalyptus oil. Different kinds of metallic ores have been found to require different oil mixtures, so that it has been necessary to redetermine 45 and readjust the proper oil mixture for each specific ore worked with.

I have discovered that the flotation process can be improved by the employment of liquid distillates from gilsonite as flotation 50 or froth-producing reagents. Not only do such gilsonite distillate reagents have good efficiency in flotation, but they are unique in their general suitability for the treatment of metallic ores susceptible of being

dealt with by flotation: in other words, 55 they are practically a universal flotation agent. They differ essentially from all oils hitherto used (singly or in admixture) in having inherently the ratio between saturated and unsaturated hydrocarbons proper 60 for flotation purposes. The consumption of oils in flotation is so large, moreover, that the applicability of a relatively cheap product such as gilsonite distillate to this use is 65 of great economic importance, since it affords the industry a possibility of largely or entirely dispensing with the use of costly agents such as pine oils, eucalyptus oil, etc., which are practically indispensable when petroleum and coal tar oils are employed 70 for flotation.

Gilsonite is a hard, brittle, shiny, black bitumen which is found in large quantity in Utah, U. S. A., and elsewhere. It occurs as veins in the earth, generally between 75 rocks, and is remarkably pure in its native state. Its specific gravity is about 1.04; the color of its powder is brown; it melts when heated. It has been used, (even in its native state) in the manufacture of black 80 varnishes and of rubber substitutes; also, by melting it or dissolving it in oils, for various other purposes.

When distilled, gilsonite yields from 8 to 10% of combustible and luminous gases and 85 ammonia, 60 to 70% of liquid hydrocarbons, and from 25 to 30% of a residue of coke. The liquid hydrocarbons obtained by distillation have a specific gravity of from .85 to .95 and are decidedly liquid at ordinary 90 normal atmospheric temperatures. They begin to boil at some 165° F., (about 75° C.), and they all distill at temperatures below some 750° F., (about 400° C.). They possess a very characteristic pungent odor, 95 difficult to define, but quite recognizable by those skilled in the art. They are characterized by a very high proportion of unsaturated hydrocarbon.

Gilsonite distillate suitable for use as a 100 flotation agent in accordance with my present invention may be obtained from gilsonite as follows:

Native gilsonite consisting of "run of mine" (both lumps and powder) is charged 105 into a steel still set over a fire box and connected with a condensing system of water or air-cooled pipes. The charge of gilsonite

may vary from 500 pounds to several tons, depending upon the capacity of the available still. The still being entirely closed (except for the opening into the condenser), a fire is started under the still,—with coal, oil, or gas fuel,—and the temperature of the gilsonite is raised gradually. As the heat is thus gradually applied, the gilsonite will liquefy and collect in the bottom of the still, and vapor and gas evolving from it will fill the top of the still and pass over into the condenser. As the heating progresses, temperature reading may be taken from time to time on the body of vapor in the upper portion of the still, as well as on the body of liquid beneath it. Excepting as there may be special occasion for distinguishing them, here and hereinafter comprehend mingled gases and vapors under the single term "vapor," for the sake of brevity. For convenience, I refer to various stages of operations by the corresponding vapor temperatures, unless otherwise specially noted.) The effect of the progressive heating of the gilsonite is to gradually break it up and decompose it,—whence, mainly, the evolution of vapor. It is a difficult matter to describe the process, or to determine in what order various products are formed or come off, since the coming off of particular products depends on the stability under heat of the highly complex chemical combinations amongst the constituents of gilsonite, as well as upon the boiling points of the products themselves. The matter is further complicated, no doubt, by the liberation, formation, and decomposition of intermediate products both in the body of liquid and in the body of vapor. However, the coming off of vapor from the still begins at a temperature of some 165° F., (about 75° C.) and continues up to or even beyond coking temperatures. The distillation may proceed, therefore, with evolution of gases and liquids, until the bottom of the still is a cherry red and the vapor temperature is some 750° F., (about 400° C.). The maximum temperature of the coke formed in the bottom of the still need not exceed some 850° F. (about 455° C.).

Up to the point where the vapor temperature approaches some 550° F. (about 285° C.), the distillation may be carried out as rapidly as the contents of the still can be made to absorb heat. At this point, however, some exothermic or other peculiar action occurs, so that the evolution of vapor in the still tends to become excessively rapid. Unless, therefore, the previous heating has been especially slow, it is advisable to reduce the application of heat very greatly as this critical point is approached, in order that undistilled liquid may not be carried over into the condenser, and clog it up so as to render it unusable. In practice, it

will usually be found convenient to cut down the fire some 100° F. in advance of this temperature. Once this critical point is well passed, the fire may be increased and the distillation pushed on as rapidly as desired to its conclusion. 70

The distillation may be entirely dry; or, if preferred, live steam may be conducted through the gilsonite in the still during the distillation. Such employment of steam is 75 advantageous, though not essential, to the process.

While the vapor coming off from the still may all be led into the iron pipe condenser, as above suggested, and all of the strictly vaporous portion thereof condensed and collected as a liquid, a slightly different procedure is preferable. A minor portion of the vapor is condensable at relatively high temperatures; and at the lower temperatures in the condenser (especially if water-cooled), the corresponding condensate is of such thick, gummy consistency that it would tend to clog it up. It is desirable, therefore, that this heavier portion of 90 the normally liquid products be condensed and collected separately, without entering the condenser at all. This can advantageously be taken care of by making the pipe leading from the still to the condenser 95 of substantial length and providing it with a trap. With this arrangement, the heavier portion of the normally liquid products will be condensed by the cooling effect of the atmosphere upon the pipe (which thus acts as a sort of auxiliary condenser), and will collect in the trap, whence it can be drawn off from time to time and added to the liquid products drawn from the condenser itself. The trap also affords a measure of protection against the effects of too rapid heating at the critical temperature above mentioned. 100

The truly gaseous portion of the distillation products will pass uncondensed through the condenser and be collected separately, in any suitable manner. The liquid condensate may be collected in any kind of suitable receiver. 110

The distillate of liquid hydrocarbons thus obtained from gilsonite may be used in metallic separation by flotation without any change or any admixture of other oils. In practicing my flotation process with it, I, therefore, add such gilsonitic distillate to 120 a watery mixture consisting of a finely pulverized metallic ore or slime and an excess of water, contained in a suitable receptacle. The mixture being constantly agitated, with air or by mechanical means, the hydrocarbons cause a froth in and on the liquid which foams over the top of the vessel (or out of an opening in one side thereof, provided for this purpose), carrying with it the metallic 125 portions of the ore under treatment and 130

leaving the gangue behind. The amount of liquid hydrocarbon required is variable, depending upon the kind of ore treated, but in general is from one-fourth of 1% to 1%.  
5 The crude distillate obtained as described above contains from 2% to 5% of water, which (though innocuous to its use as a flotation reagent) may readily be eliminated by settling out in a settling tank. The distillate is a reddish brown oil with a green fluorescence; it is decidedly liquid at ordinary atmospheric or normal temperatures; is of about 0.875 specific gravity at 60° F., (about 15° C.); begins to boil near the lower limit (165° F., or about 75° C.) of the temperature range mentioned above, and distills completely below the upper limit (some 750° F., or about 400 C.) of said range; flashes in the air at ordinary temperatures; and contains, (as already mentioned), a very high percentage of unsaturated hydrocarbons, usually about 60%. It is immiscible and insoluble in water, but completely soluble in benzole and carbon-bisulphide, and miscible in all proportions with petroleum and petroleum products, and with turpentine and with pine oil.

While the crude primary gilsonite distillate obtained as described above may be used directly as a flotation reagent, yet, if desired, certain light hydrocarbons that are otherwise very useful may be removed from the crude distillate without impairing the fitness and advantages of the residue for flotation. For example, a dry redistillation or reduction may be carried out in a suitably heated steel still, the vapors coming off up to some 600° F., (about 315° C.) vapor temperature being condensed, with incidental fractionation, if desired, and the residue of oil unvaporized at 600° F. being subsequently drawn off for use as flotation reagent without further treatment of any sort.

This heavy residual oil redistillate may have a specific gravity of as high as 0.933; it is a somewhat viscous reddish-yellow oil with green fluorescence when freshly prepared, but on standing becomes black in the mass and brown in a thin film; and it is as well suited for flotation purposes as the lighter primary crude distillate, or even better.

I make no claim of novelty for the apparatus referred to in the above description of the production of gilsonitic distillate; on the contrary, practically any type of destructive distillation apparatus may be employed which will produce such distillate from gilsonite. Neither do I here claim the distillation process described above, nor the gilsonitic distillates thereby produced, since all these and other matters here disclosed or referred to form the subject of my pending applications, Serial No. 195,721 of October 10, 1917 (above mentioned), and Serial No. 318,536 of August 19, 1919, entitled "Gilsonite products and their manufacture."

Having thus described my invention, I claim:

The process of metallic separation, which consists in adding to a watery mixture containing finely pulverized ores or slimes a liquid hydrocarbon obtained from the destructive distillation of gilsonite and characterized by a very high percentage of unsaturated hydrocarbons; and aerating the mixture, whereby the metallic portions of the ore are separated from the gangue.

In testimony whereof, I have hereunto signed my name at Maurer, N. J., this 6th day of November, 1920.

CHARLES N. FORREST.

Witnesses:

DENNIS J. DESMOND,  
CHARLES HARNED.